

# UNITED STATES PATENT OFFICE.

HERMANN G. C. THOFEHRN, OF NEW YORK, N. Y., ASSIGNOR TO LIGHT METALS CO.,  
OF ELIZABETH, NEW JERSEY.

## ALLOY.

1,310,309.

Specification of Letters Patent. Patented July 15, 1919.

No Drawing.

Application filed December 15, 1917. Serial No. 207,311.

*To all whom it may concern:*

Be it known that I, HERMANN G. C. THOFEHRN, a citizen of the United States, and a resident of New York, in the county of 5 New York and State of New York, have invented certain new and useful Improvements in Alloys; and I do hereby declare the following to be a full, clear, and exact 10 description of the invention, such as will enable others skilled in the art to which it appertains to make and use the same.

This invention relates to an improvement in alloys,—the object of the invention being to produce an alloy which shall be exceedingly 15 light in weight and at the same time possess great tensile strength and toughness, with sufficient elasticity to render the same of great value in the manufacture of structural work in which such qualities, in a high 20 degree, are essential.

With this object in view, the invention consists of an alloy having the composition of metals hereinafter set forth and pointed out in the claims.

25 My improved alloy comprises aluminum, magnesium and uranium in approximately the following proportions; to wit, aluminum from 94 to 98 per cent., magnesium from 2 to 6 per cent. and uranium from 0.01 to 0.3 30 per cent.

In the manufacture of the alloy, I proceed as follows: I first place in a suitable crucible or container a quantity of uranium oxid sufficient to provide in the finished alloy a 35 uranium content of from 0.01 to 0.3 per cent., and apply heat to raise the temperature of the said uranium oxid to a bright red heat. I then introduce aluminum in the proportion of from 94 to 98 per cent. and 40 when the mass has become molten, I add magnesium in the proportion of from 2 to 6 per cent. As these molten metals react upon the uranium oxid, the latter will be reduced to metal which is dissolved throughout 45 out the whole mass.

In order to avoid the metal retaining gases which would make it porous, I agitate the molten mass with the use of an iron rod having a disk of iron on one end. With the use of this tool, I perform a pumping action 50 in the molten mass, agitating the same gently and causing the disk or headed end of the tool to remain under the surface of the mass to avoid splashing. Such gentle agitation will cause gases which may be contained in the molten metal to escape, and thus a good sound casting may be obtained. 55

By means of my improved process, I obtain an alloy which is of exceedingly light weight but having great tensile strength and 60 toughness and which is eminently suitable in the manufacture of structural work where a maximum of such qualities is an important consideration.

Having fully described my invention what 65 I claim as new and desire to secure by Letters-Patent, is:—

1. An alloy having great tensile strength and toughness and light in weight, composed of aluminum, magnesium and uranium, the major portion of the alloy composed of aluminum and the magnesium and uranium being in relatively small proportions. 70

2. An alloy consisting essentially of aluminum, magnesium and uranium, the aluminum being approximately from 94 to 98 per cent., the magnesium approximately from 2 to 6 per cent., and the uranium approximately from 0.01 to 0.3 per cent. 75 80

In testimony whereof, I have signed this specification in the presence of two subscribing witnesses.

HERMANN G. C. THOFEHRN.

Witnesses:

DONALD H. MCLEAN,  
VIVIAN L. ADELBERG.